

June 8, 1926.

1,588,226

E. F. HOLINGER

METHOD OF MAKING GATE VALVES AND SIMILAR BODIES

Filed Oct. 2, 1924

Fig. 1.



Fig. 2.



Fig. 3.



Fig. 4.



Fig. 5.

INVENTOR.

EMIL F. HOLINGER.

BY *Sheffield & Betts*  
HIS ATTORNEYS

## UNITED STATES PATENT OFFICE.

EMIL F. HOLINGER, OF JERSEY CITY, NEW JERSEY, ASSIGNOR TO THE M. W. KELLOGG COMPANY, OF NEW YORK, N. Y., A CORPORATION OF DELAWARE

## METHOD OF MAKING GATE VALVES AND SIMILAR BODIES.

Application filed October 2, 1924. Serial No. 741,202.

This invention relates to a method of making gate valve bodies from steel and similar materials in which a solid billet or ingot is formed by drop forging, hydraulic forging or in any other suitable way into the desired form, holding the formed ingot in a suitable die conforming to the exterior shape to be produced and forming opposing valve seats and the neck of the valve by 10 placing the metal with a punch through an opening in the side of the die.

An object of my invention is to provide a simple and efficient method whereby devices of this character may be readily and 15 economically manufactured.

My invention will be better understood from the following description taken in connection with the accompanying drawings and its scope will be pointed out in the appended claims.

In the drawings illustrating my invention:

Fig. 1 is a side view of one type of the forging.

Fig. 2 is a side view of another type of the forging.

Fig. 3 is a view of the punching apparatus with parts broken away showing the die in vertical section with a forging therein in elevation.

Fig. 4 is a vertical longitudinal sectional view of a valve casing as it leaves the punching apparatus, and Fig. 5 is a plan view of the valve casing of Fig. 4.

Referring to the drawings in which the numeral 1 indicates a solid billet or ingot which has been formed by drop forging, hydraulic forging or in any other suitable way, into the desired shape. To illustrate my invention, I have shown a forging having a relatively large central mass indicated at 2, with lateral cylindrical portions 3, 4, extending from opposite sides. The precise form of the forging is not material, but it is desirable that the part 2 which is to be pierced to form the valve seats be of sufficient mass for displaced metal to form the valve neck. The mass 2 may be formed with a small lower end 2' extending beyond the lower edges of parts 3 and 4, as shown in Fig. 1, or the parts 3 and 4 may constitute the body of the forging with the mass 2 positioned on one side of their center line,

as shown in Fig. 2. The mass 2 may assume many different forms. The forging 1, 55 which may be either of the types shown, or other suitable types, is placed in a split die 5 conforming to the exterior shape of the forging and with such additional conformations as are desired on the article to be 60 produced. The lower part 6, of die 5, is provided with a suitable depression 7 centrally positioned with respect to central mass 2 of forging 1 in which the lower part of the valve casing is formed. The upper 65 part 8 of die 5 has a central opening 9, of any desired shape, preferably circular in cross-section and in alignment with the depression 7. The shape and size of the valve neck is determined respectively by the cross- 70 section contour and by the diameter of opening 9. The opening 9 is positioned below a punch or piercing tool 10, operated by hydraulic or mechanical pressures or other suitable means, not shown in the drawings, and 75 may be supported by the upright bars or posts 11 if desired. The punch or tool 10 in the present instance is circular in cross-section at its upper end and of smaller diameter than opening 9 of die 5, the difference in sizes determining the thickness of the wall of the valve neck. The lower end 80 of tool 10 is cut away on opposite sides as shown at 11, 12, at an angle tapering toward the lower end and small shoulders are formed at 13, 14. Opposite each other and between the cut away parts, the tool 10 is 85 provided with grooves, one of which is shown at 15.

After the forging 1 has been placed 90 within die 5 as shown in Fig. 3, the piercing tool 10 is forced into the die under heavy pressure, which causes the material of the ingot to flow into the depression 7 and upwardly around the tool 10 forming a 95 valve neck between the wall of die opening 9 and the part of the tool above shoulders 13, 14. As shown in Figs. 4 and 5, the forging 1 has now been formed with opposing valve seats 16, 17, part 7', a valve 100 neck 18, shoulders 19, 20 within the valve neck at the lower end thereof and inner guide flanges 21 and 22. An opening, as indicated in dotted lines at 23, may now be 105 drilled or bored through the body thus formed in any suitable manner, and the

neck 18 may be threaded as indicated in dotted lines at 24.

From a consideration of the above description, taken in connection with the drawings, my invention will be apparent without further description. I do not wish to be understood as being limited to the details of form or arrangement of parts herein set forth, for various changes may be made by those skilled in the art without departing from the spirit or scope of my invention.

What I claim and desire to protect by Letters Patent is:

1. The method of making gate valve bodies from steel and similar materials which comprises first forming a solid ingot into substantially the external shape of the valve body by forging, holding the same in a die having a lateral opening, forcing a punch into said die through said opening, said punch having a portion adapted to form opposing valve seats and another portion adapted to form the neck of the valve, thereby causing the metal to be displaced and flow into the upper portion of said die to form the neck of the valve, and then cutting a passage through the connecting portions of said valve body.

2. The method of making gate valve bodies from steel and similar materials which comprises first forging an ingot into substantially the external shape of the valve body, holding the solid forging in a suitable die conforming to the exterior shape thereof, said die having a lateral opening, and then forming opposing valve seats and a neck on said solid body by piercing the same through said lateral opening with a punch having valve seats and valve neck forming portions thereon, thereby causing displaced metal to flow into said neck portion of said die to form the valve neck in

said lateral opening, and then cutting a passage through the connecting portions of said valve body.

3. The method of making gate valve bodies from steel and similar materials which comprises first forging a solid ingot into substantially a valve body having an enlarged central mass, holding the ingot in a correspondingly shaped die having a lateral opening, the enlarged mass being positioned below said opening, and forcing a punch into the die through said opening, said punch having a tapering portion adapted to form opposing inclined valve seats and another portion adapted to form the neck of the valve, thereby causing the metal from the mass to be displaced and flow into the upper portion of said die to form the neck of the valve, and then cutting a passage through the connecting portions of said valve body.

4. The method of making gate valve bodies from steel and similar materials which comprises first forging a solid ingot into substantially a valve body having a central enlarged portion and oppositely extending fully shaped members, holding the ingot in a correspondingly shaped die having a lateral opening, the central mass being below said opening, and forcing a punch into said die through said opening, said punch having a wedge-shaped portion adapted to form converging valve seats and another portion adapted to form the neck of the valve, whereby the metal will flow from the central mass into the upper portion of said die to form the neck of the valve, and then cutting openings through said oppositely extending members to communicate with the valve seats and neck so formed.

EMIL F. HOLINGER.